

## UNITED STATES PATENT OFFICE

2,513,237

METHOD OF PROTECTION OF MAGNESIUM  
AND MAGNESIUM-BASE ALLOYSHerbert Manfred Freud dit Jean Frasch,  
Nanterre, FranceNo Drawing. Application July 23, 1947, Serial  
No. 763,159. In France September 22, 1938

9 Claims. (Cl. 204—56)

1

The present invention concerns the treatment of objects made of magnesium metal or alloys composed principally (e. g. 85% or more) of magnesium, for forming on said objects a film or coating which can protect said articles from corrosion. As is well known, magnesium in the pure state and to a somewhat less extent alloys which contain magnesium associated (alloyed) with small amounts (up to 10% or 15%, more or less) of other common metals, e. g. Mn, Zn, Al, rare earth metals, etc., are prone to become oxidized or corroded by continued exposure to damp air, air containing traces of acid vapors, air containing moisture and salts, or sea water, river water, lake water, etc., and efforts have long been made to protect such magnesium or magnesium alloys, from such oxidation and corrosion. The present invention covers such protection.

Hereinafter, the term "magnesium-base metal" will be used to cover such metal and alloys as discussed above.

The objects may be cast, forged, machined, rolled, etc. and may be of any appropriate sizes and may be completely made, or not, as desired. The articles (unless already wholly clean) should first be degreased, cleaned, washed and dried, which steps may be carried out according to processes already known.

The present invention is in part a continuation of my earlier application Ser. No. 297,191, filed Sept. 29, 1939, (which has become abandoned).

The present process involves an alternating current electrolytic treatment, in a bath of proper acidity, consisting principally of an aqueous solution of manganese dichromate, free from substances capable of attacking the magnesium in such a way as to bring any magnesium compounds into the coating being formed on the objects treated, and/or to bring any substantial amount of magnesium compounds into solution in the electrolytic bath. Coatings of the type set forth herein, which contain magnesium compounds (oxide or salts) are usually porous and only insecurely attached to the object treated, are generally weak and offer only slight protection. This is because MgO is to a slight extent capable of being dissolved by water, especially water containing usual amounts of carbon dioxide in solution. Most so-called "insoluble" magnesium salts are likewise subject to attack by water, especially water containing usual amounts of carbon dioxide in solution.

It is important, in order to avoid chemical attack of the magnesium, with consequent introduction of such magnesium compounds into the

electrolyte and/or into the coating being formed on the object, to avoid the presence in the electrolyte of any substantial amounts of acids which would chemically attack magnesium, to dissolve the same, such acids as sulphuric, phosphoric, nitric, hydrochloric, and many of the common organic acids, in any substantial amounts, thus being excluded from the electrolyte, as well as the salts of such acids. But mere slight traces of such acids, even of the strong mineral acids, do no appreciable harm, and hence can be tolerated. Hence it is not necessary, in making up the electrolyte to use the substances (CrO<sub>3</sub>, MnCO<sub>3</sub>, MnO<sub>2</sub>, etc.) in an absolutely chemically pure state, but the amounts of impurities therein, especially sulphates, halides, etc., should not be great. The definite addition of substantial amounts of sulphates, phosphates, nitrates, halides, etc., of course is avoided.

It is of course understood that while I preferably use two articles or objects of magnesium-base metal as the two electrodes, and these two articles are preferably alike and have equal surface areas, it is permissible to use such a magnesium object as one electrode with an insoluble electrode of electrically conductive material such as carbon, with the production of equally good results.

In carrying out the process, the electrolyte is a solution of manganese dichromate, MnCr<sub>2</sub>O<sub>7</sub>. This solution should have a pH between 2 and 5, and preferably between 3 and 4. A pH of close to 3.5 is preferable and produces the best results.

This solution is preferably made by dissolving 10 to 100 grams of chromic anhydride, CrO<sub>3</sub> in a liter of water, and adding manganese carbonate thereto, to give the desired pH. The CO<sub>2</sub> of the carbonate is liberated into the atmosphere. Hence the carbonic acid does not act to injure the magnesium. Manganese dioxide, preferably in a freshly precipitated state can be similarly dissolved in the chromic acid solution, preferably heated. A part of the oxygen content of the dioxide is liberated during the reaction. Manganese oxalate can be used in a similar manner, this also liberating CO<sub>2</sub> (chromic acid being a strong oxidizer). In this latter case, solution is preferably effected, hot. Mixtures of the manganese compounds can also be used. Manganese carbonate is the preferred compound to use.

Manganese carbonate, MnCO<sub>3</sub> is readily obtainable, is relatively cheap and is easily and promptly dissolved by chromic acid solutions and the action of the chromic acid thereupon can

take place effectively at ordinary atmospheric temperatures. Preferably the carbonate is added to the chromic acid solution in such amount as to form a manganous dichromate solution having a pH of 3.5. For best results I add about 6.25 parts by weight of  $MnCO_3$  to each 10 parts of  $CrO_3$  in the solution, both ingredients being of commercial purity.

The ratio of the manganese carbonate to  $CrO_3$ , in order to give the best results is within the range 5 to 7 parts (preferably 5.5 to 6.5) of manganese carbonate to 10 parts  $CrO_3$ . This same proportion (2.4 to 3.4 parts of the element manganese to 10 parts  $CrO_3$ , and preferably 2.6 to 3.1 parts of the element manganese to 10 parts  $CrO_3$ ) will be observed using the other manganese compounds named above as the source of manganese ions.

Normal manganese chromate  $MnCrO_4$  is not readily soluble in water. Manganese dichromate  $MnCr_2O_7$  is sufficiently soluble. It will be understood that the ratio of manganese compound to  $CrO_3$  as set forth herein is about the proper proportion for the formation of the  $MnCr_2O_7$ , with perhaps a slight excess of  $CrO_3$ . The electrolyte may contain between 2.66% and 12% (e. g. 4% to 10%) of manganese bichromate (based on the whole electrolyte). Without limiting the invention to the details, I give the following examples:

Two electrodes (each a machined plate-like object of magnesium metal), of approximately equal size and equal surface area are immersed in a bath made from 7.5 parts  $CrO_3$  and 4.7 parts  $MnCO_3$  in 100 parts of solution. This gives a substantially 10% solution of manganese bichromate,  $MnCr_2O_7$  (perhaps combined with some water). The two electrodes were connected to the A. C. circuit, at 15 volts, and an alternating current of 4 amperes per square decimeter was allowed to flow through the cell for about 15 minutes. The electrolyte was at room temperature (about 18-20° C.), throughout said treatment. At the end of this period, the electrodes were removed from the solution, well washed in running water, dried and examined. It was found that the objects had a strongly adhering deposit covering their surfaces, which was dark brown, nearly black in color, composed of  $CrO_2$  and  $Mn_3O_4$ . This coating offered good protection against corrosion. The coating is not porous.

The coating on the magnesium was quite impervious to water and aqueous solutions. The so coated articles could be given coats of oil paint, varnish, lacquer, etc. to afford long-lasting protection.

It is also possible to somewhat vary the proportion of  $MnCO_3$  and  $CrO_3$  used in making the electrolyte, to give pH values between 2 and 5. The coatings are less good as the pH of the electrolyte is above or below the optimum of 3.5. With lower pH, the coatings are somewhat more porous. This can be somewhat offset by a good painting.

The coatings can also be somewhat improved by a subsequent boiling in sodium silicate solution or by treatment in hot molten paraffin, as shown in my copending patent applications.

The strength of the alternating current can vary between 1.5 and 12 amperes at a voltage between 4 and 40 volts. The duration of the A. C. electrolytic treatment can vary substantially. A treatment for 15 to 20 minutes is usually sufficient to give a sufficiently thick coating.

I also give the following specific examples which have shown favorable results.

(a) 100 gr.  $CrO_3$ , 65 gr.  $MnCO_3$ , 1 liter of water. This gives a substantially 12% solution of manganese bichromate. A. C. treatment at 15 volts, 4 amperes per square decimeter of surface of magnesium or magnesium-base alloy object treated, continued 15 minutes at 15-20° C.

(b) 20 gr.  $CrO_3$ , 12 gr.  $MnCO_3$ , 1 liter of water. This gives a substantially 2.66% solution of manganese bichromate. A. C. at 18 volts, 3 amperes per sq. decimeter of Mg. surface, continued 15-20 minutes at 15 to 20° C.

I claim:

1. A process of protecting magnesium-base metal objects in an electrolyte which consists essentially of an aqueous solution which is the liquid reaction product made by dissolving at least one substance selected from the group consisting of manganese carbonate, manganese dioxide and manganese oxalate, which substance contains from about 2.4 to about 3.4 parts by weight of the element manganese, in an aqueous solution of chromic acid alone, containing the equivalent of 10 parts by weight of chromic anhydride in about 100 to 1,000 parts by weight of water, and applying said liquid reaction product, while the latter is free from more than traces of acids which are capable of chemically attacking metallic magnesium and dissolving same, and free from more than traces of salts of such acids, and while such solution has a pH value between about 2 and about 5, as an electrolytic bath, in which is placed a pair of electrodes, at least one of which is such a magnesium-base metal object and the other electrode being formed of an electrically conductive material which is insoluble in said electrolyte, and applying to such electrodes an alternating electric current of between 1.5 and 12 amperes per square decimeter of surface of said magnesium-base metal object being treated, at a voltage between 4 and 40 volts, at about atmospheric temperature, and continuing the treatment until a good protective film substantially free of magnesium compounds has been formed on said magnesium object.

2. A process of protecting magnesium-base metal objects which comprises dissolving a substance selected from the group consisting of manganese carbonate, manganese dioxide and manganese oxalate, which substance contains about 2.6 to about 3.1 parts of the element manganese, in an aqueous solution of chromic acid alone, containing the equivalent of 10 parts of chromic anhydride, and applying said solution, while the latter is free from more than traces of acids which are capable of chemically attacking metallic magnesium and dissolving same, and free from more than traces of salts of such acids, and while such solution has a pH value of about 3.5, as an electrolytic bath in which is placed a pair electrodes, at least one of which is such a magnesium-base metal object and the other electrode being formed of an electrically conductive material which is insoluble in said electrolyte, and applying to such electrodes an alternating electric current of about 4 amperes per square decimeter of surface of said magnesium-base metal object being treated, at a voltage of between 10 and 20 volts, at about room temperature, and continuing the treatment until a good protective film has been formed on said object.

3. A process as claimed in claim 1 in which a pair of said magnesium-base objects, having about

equal surface areas, constitute the two electrodes in said electrolytic bath.

4. A process which comprises applying an alternating electric current to an electrolytic cell containing a pair of electrodes in an electrolyte, at least one of said electrodes being an object composed of magnesium-base metal, and the other electrode being an electrically conductive material which is insoluble in said electrolyte, and in which said electrolyte consists essentially of an aqueous solution of manganese dichromate having a pH value between about 2 and about 5, which solution is free from more than traces of acids which would be capable of chemically attacking metallic magnesium and dissolving same, and free from more than traces of salts of such acids, the said alternating electric current being between about 1.5 and 12 amperes per square decimeter of surface of said magnesium-base metal object being treated, and at a voltage between about 4 and about 40 volts, and continuing said treatment until a good protective film has been formed on said object.

5. A process as in claim 4, in which the pH of the electrolyte is about 3.5.

6. For protecting magnesium base articles against corrosion, the step of subjecting such an article, as an electrode, to alternating current electrolysis in a bath consisting essentially of an aqueous solution of manganese bichromate, and which bath has a pH between 3 and 4, which bath is substantially free of acids which can chemically attack metallic magnesium and substantially free of the salts of such acids.

7. For protecting magnesium base articles against corrosion, the step of subjecting such an article, as an electrode, to alternating current electrolysis in a bath consisting essentially of an aqueous solution of manganese bichromate of about 4% to about 10% concentration, and which bath has a pH between 3 and 4, which bath is substantially free of acids which can chemically attack magnesium and substantially free of the salts of such acids.

8. For protecting magnesium base articles against corrosion, the step of subjecting such an article, as an electrode, to alternating current electrolysis in a bath consisting essentially of an aqueous solution of manganese bichromate of about 2.66% to about 12% concentration, and which bath has a pH between 3 and 4, which bath is substantially free of acids which can chemically attack magnesium and substantially free of the salts of such acids.

9. In protecting magnesium base metal articles, by A. C. electrolysis in an acid chromate solution, the steps of forming the electrolyte by heating manganese oxalate in a liquid consisting essentially of water and chromic acid until carbon dioxide is liberated, the ratio of chromic acid to manganese oxalate being such as to leave an aqueous solution containing manganese bichromate, and applying alternating electric current to electrodes, at least one of which is magnesium-base metal, while immersed in said aqueous solution as electrolyte.

HERBERT MANFRED FREUD

BY JEAN FRASCH.

#### REFERENCES CITED

The following references are of record in the file of this patent:

#### UNITED STATES PATENTS

| Number    | Name    | Date          |
|-----------|---------|---------------|
| 2,114,734 | Buzzard | Apr. 19, 1938 |
| 2,206,028 | Buzzard | July 2, 1940  |
| 2,463,483 | Frasch  | Mar. 1, 1949  |

#### FOREIGN PATENTS

| Number  | Country | Date          |
|---------|---------|---------------|
| 702,266 | France  | Jan. 20, 1931 |
| 832,002 | France  | June 20, 1938 |
| 377,355 | Italy   | Dec. 16, 1939 |

#### OTHER REFERENCES

"Metaux & Corrosion," vol. 14, No. 166 (June 1939), pages 83 through 87.